

Patented Feb. 28, 1933

Barium hydrate as  
a binder 1,899,152

## UNITED STATES PATENT OFFICE

WILLIAM E. JEAVONS, OF CLEVELAND HEIGHTS, AND MAHON J. RENTSCHLER, OF  
WILLOUGHBY, OHIO

## PROCESS OF CONDITIONING INCOHERENT FINELY DIVIDED MATERIALS

No Drawing.

Application filed November 14, 1930. Serial No. 495,780.

This invention relates to a method of conditioning finely divided incoherent materials whereby these materials may be rendered available for use in the industrial arts. An instance of such materials is barium peroxide which, as is well known, is ordinarily a finely divided incoherent powder. It has been proposed to use barium peroxide in the treatment of molten metal, such as steel, but it has been found impracticable to do so because of the fact that, when applied to the molten steel, it floats on the surface of the charge, the resultant reaction being so extremely rapid that only a small portion of the mass is affected thereby. Under ordinary conditions, the molten steel is covered with a coating of slag and, when barium peroxide in its ordinary form is introduced into a furnace containing such melted charge, it does not penetrate the slag coating and hence has no effect whatever upon the steel.

We have found that, by incorporating (where necessary) a small proportion of barium oxide with the barium peroxide and in thorough admixture therewith, and by thoroughly mixing with such mass a small quantity of cold water—in no greater quantity than is necessary to convert the barium oxide into completely crystallized barium hydrate—an efficient binder is formed whereby the mass may be molded under pressure and compacted into an integrated body, such as a briquette. The addition of cold water does not affect the barium peroxide; but it produces, by reaction with the barium oxide, crystallized barium hydrate which forms a most effective binder and enables the mixture to be compacted in the manner described. The barium hydrate acts as a setting agent, in addition to binding the mass, whereby a body molded as described retains its solidity and the barium peroxide retains its full strength, even where the bodies are kept in storage for a considerable length of time. Furthermore, when exposed to high temperatures, the bodies produced in the manner described do not disintegrate. When introduced into or applied to a mass of molten metal, the body containing barium peroxide prepared in the manner described possesses

sufficient density to be partially submerged in the molten metal below the slag line, thus enabling the barium peroxide to contact in a most efficient manner with the molten metal. The reaction between the molten metal and the barium peroxide takes place gradually, the decomposition proceeding from the outside of the body inwardly and the body sinking into the molten metal as decomposition proceeds—in a manner similar to that which occurs through the melting of ice in water. During this gradual decomposition, the interior of the body retains its strength or reactivity; and it is obvious that the period of reaction between the barium peroxide and the molten metal is greatly prolonged to an extent and in a manner which will enable the barium peroxide to react most effectively with the impurities in the metal.

While the use of barium oxide as a binding and cementing agent has proved to be of great value in the conditioning of barium peroxide, it will be obvious that it may be used with beneficial results in the conditioning of other materials which are normally in the form of finely divided incoherent powder. For instance, it has been beneficial in the treatment of finely divided ores, carbon blacks, and lamp blacks, which are very bulky and which offer great difficulties in transportation. It is, of course, obvious that materials that will be affected adversely by chemical reaction with barium oxide should not be integrated thereby. However, our experiments show that it may be used with pigments and generally wherever the barium oxide will not set up any adverse chemical reaction with the material with which it is used. In each of the instances mentioned, the presence in the compacted bodies of material of the small proportion of barium hydrate does not interfere with the intended use thereof.

In some cases, it is preferable to encase the bodies thus formed in cases or cartridges, preferably of sheet metal, in order to protect the bodies from erosion in transportation and in the rough handling to which they are subjected in mill practice. This is particularly true where the bodies are to be used

for the treatment of molten metal, where the cases or cartridges will be quickly melted away from the bodies or otherwise removed by the action of the heat thereon.

Having thus described our invention, what we claim is:

1. The process of conditioning incoherent finely divided substances which consists in adding to a mixture of the same and a small proportion of barium oxide, just sufficient cold water to convert the barium oxide into barium hydrate, and forming the resultant mass into one or more integrate bodies.
- 15 2. The process of conditioning barium peroxide for the treatment of molten metal which consists in forming a mixture of the same with a small proportion of barium oxide, adding sufficient cold water to the mixture to convert the barium oxide into barium hydrate, and compressing the resultant mass into one or more integrate bodies.
- 20 3. The process of conditioning incoherent material reactive to molten metal which consists in forming a mixture of such material with a small proportion of barium oxide, adding just sufficient cold water to the mixture to convert the barium oxide into barium hydrate, and compressing the resultant mass into one or more cartridges or casings which
- 25 30 will be removed by the heat of the molten metal.
4. The process of conditioning barium peroxide for the treatment of molten metal which consists in forming a mixture of the same with a small proportion of barium oxide, adding sufficient cold water to the mixture to convert the barium oxide into barium hydrate, and compressing the resultant mass into one or more cartridges or casings capable of being removed by the action of the molten metal.
- 35 5. The process of conditioning barium peroxide for the treatment of molten metal which consists in forming a mixture of the same with a small proportion of barium oxide and cold water and compressing the resultant mass into one or more integrate bodies.

In testimony whereof, we hereunto affix  
50 our signatures.

WILLIAM R. JEAVONS.  
MAHLON J. RENTSCHLER.